# EUROPEAN PATENT SPECIFICATION

(11) **EP 0 557 796 B1**
(45) Date of publication and mention of the grant of the patent: **11.06.1997**
(21) Application number: 93102037.4
(22) Date of filing: 10.02.1993
(51) Int. Cl.: C10M 107/00, C10M 111/04, C10M 169/04, C10M 171/00

(54) **Lubricant for refrigerating machine employing refrigerant comprising tetrafluoroethane**
Schmiermittel für Kältemaschinen,die Tetrafluoroethane als Kühlmittel verwenden
Lubrifiant pour machine frigorifique utilisant un réfrigérant contenant du tétrafluoroéthane

(30) Priority: 18.02.1992 JP 30528/92
(43) Date of publication of application: 01.09.1993
(73) Proprietor: IDEMITSU KOSAN COMPANY LIMITED, Tokyo 100 (JP)
(72) Inventor: Katafuchi, Tadashi, c/o Idemitsu Kosan Co., Ltd., Ichihara-shi, Chiba-ken (JP); Nakamura, Akira, c/o Idemitsu Kosan Co., Ltd., Ichihara-shi, Chiba-ken (JP)
(74) Representative: Türk, Gille, Hrabal, Leifert

## Description

### BACKGROUND OF THE INVENTION

### 1. Field of the Invention

The present invention relates to a lubricant for refrigerating machines employing a refrigerant comprising tetrafluoroethane. More particularly, it relates to a lubricant for refrigerating machines which is used along with a refrigerant comprising a substitute fluorohydrocarbon (hereinafter sometimes referred to as "flon compound") such as 1,1,1,2-tetrafluoroethane (R-134a). As such, the lubricant is excellent in the performance such as wear resistance, electrical insulating properties, hydrolytic stability, nonhygroscopicity and the like and further has excellent returnability of the lubricant in a compression-type refrigerating cycle (the characteristics that the lubricant is inclined to return to a compressor after it is circulated in the refrigerating cycle).

### 2. Description of the Related Arts

Conventionally, in a compression-type refrigerating cycle comprising a compressor, a condenser, an expansion valve and an evaporator, a flon compound including a fluorinated hydrocarbon such as dichlorodifluoromethane (R-12) and chlorodifluoromethane (R-22) has been used as the refrigerant. Many kinds of lubricants compatible with them have also been produced industrially available for use.

However, there have been misgivings that these flon compounds widely used as the refrigerant are liable to cause depletion of the ozone layer and environmental pollution after they are released into the open air. In an effort to prevent environmental pollution, fluorohydrocarbons (or chlorofluorohydrocarbons), for example 1,1,1,2-tetrafluoroethane (R-134a) and the like have been developed as a possible replacement in recent years. Until now there have been introduced into market many so-called substitute flon compounds with minimized danger of environmental pollution and capable of satisfying said required properties, for example 1,1,2,2-tetrafluoroethane (R-134) and the like, as well as R-134a.

These new substitute flon refrigerants are different from conventional flon refrigerants in characteristics. Thus, glycol compounds, ester compounds and the like have been proposed as the lubricant for use in combination with them (U.S. Patent No. 4,755,316 and Japanese Patent Application Laid Open No.33193/1991), and these patents are intended to dissolve substitute flon refrigerants and lubricants completely so as to provide good returnability of the lubricants.

EP-A-0 377 122 discloses a lubricating oil for compression-type refrigerator comprising as a main component a polyoxyalkyleneglycol derivative said lubricating oil has favorable compatibility with refrigerants and an excellent lubricating property, and is utilized as the lubricating oil for compression-type refrigerator employing hydrogen-containing flon refrigerants including FLON 134a.

US-A-4 946 611 disclosed fluorinated polysiloxanes to be used as lubricant for refrigerators which use various Flon compounds as refrigerants.

In an attempt to circulate all over a refrigerating cycle a refrigerant and a lubricant in their completely dissolved state as envisaged by these patents, however, said lubricant must be selected from only a very limited number of compounds acceptable to the chemical properties of substitute flon refrigerants such as R-134a. Accordingly, the selected lubricant is forced to sacrifice certain aspects of the important performance required as the lubricant.

In fact, polyalkylene glycol compounds and ester compounds thereof, both known as compatible with R-134a, have been found to have insufficient wear resistance, along with faulty electrical insulating properties. It has also been found that the polyalkylene glycol compounds are highly hygroscopic and the ester compounds thereof are hydrolytically unstable. Thus the demand for a solution in these problems has been raised in relevant industrial segments.

The present invention has been completed on the basis of a concept quite contrary to ordinary common knowledge as set forth above, in an effort to find a solution in the problems. As the result, it has been found that all these aspects of the performance can be unified by using a substance excellent in wear resistance, insulation resistance and the like as the lubricant, compounding therewith a fluidity improver to improve the fluidity of the lubricant in the presence of a refrigerant (R-134a and the like) and thus providing good returnability of the lubricant in a compression-type refrigerating cycle. It has thus been made possible that a lubricant combined even with a new refrigerant has all the required performance including excellent wear resistance, electrical insulating properties, hydrolytic stability and the like and further ensuring excellent returnability of the lubricant. The present invention has been accomplished based on this finding.

### SUMMARY OF THE INVENTION

Therefore, an object of the present invention is to provide a lubricant for refrigerating machines employing a refrigerant comprising tetrafluoroethane, which is excellent in the performance such as wear resistance, electrical insulating properties, hydrolytic stability, nonhygroscopicity and the like and further has excellent returnability of the lubricant. The lubricant can be used along with a substitute flon refrigerant in a compression-type refrigerating cycle without a hitch.

Another object of the present invention is to provide a lubricant for refrigerating machines employing a refrigerant comprising tetrafluoroethane, which is especially effective when used in automobile or household air conditioners and refrigerators and the like, having high industrial usefulness.

The present invention provides a lubricant for refrigerating machines employing a refrigerant comprising 1,1,1,2-tetrafluoroethane or 1,1,2,2-tetrafluoroethane which comprises as an essential component a base oil comprising (A) 60 to 90% by weight of a synthetic oil formed of a poly-α-olefin or a mixture of a poly-α-olefin and an alkylbenzene and (B) 10 to 40% by weight of a fluidity improver comprising at least one compound selected from the group consisting of a polyoxyalkylene glycol compound and a polysiloxane compound.

The lubricant of the present invention can be suitably used in various refrigerating machines and ordinarily in a compression-type refrigerating cycle comprising a compressor, a condenser, an expansion valve and an evaporator.

### DESCRIPTION OF PREFERRED EMBODIMENTS

As set forth above, the lubricant of the present invention comprises the components (A) and (B) as the essential components, and the synthetic oil constituting the component (A) is a poly-α-olefin or a mixture of a poly-α-olefin and an alkylbenzene.

Various poly-α-olefins can be used and ordinarily are each a polymer of α-olefin having 8 to 14 carbon atoms and a kinematic viscosity of 10 to 350cSt at 40°C. Preferred among them is a polymer of 1-dodecene, a polymer of 1-decene or a polymer of 1-octene, each having a kinematic viscosity of 10 to 350cSt at 40°C. A lubricant containing a synthetic oil comprising such a poly-α-olefin has a lower viscosity at low temperatures in the presence of a tetrafluoroethane refrigerant, and thus returnability of the lubricant is all the more improved.

Various alkylbenzenes can be used as well and ordinarily are each an alkylbenzene having a kinematic viscosity of 5 to 500cSt, preferably 10 to 350cSt at 40°C. Meanwhile, either soft or hard alkylbenzene can be used provided that it meets this condition.

The alkylbenzene is not used singly but in the form of a mixture thereof with said poly-α-olefin as the synthetic oil as the component (A) in the present invention. The mixing ratio of the poly-α-olefin to the alkylbenzene may be appropriately selected according to circumstances and is not particularly limited. Preferably the mixture has a poly-α-olefin content of 5% or more by weight, more preferably 5 to 90% by weight, most preferably, when using high viscosity poly-α-olefin having a kinematic viscosity of about 50cSt or more at 40°C, 5 to 50 % by weight of the mixture. When such a mixture of the poly-α-olefin and alkylbenzene is used as the synthetic oil as the component (A), the mixing stability of the poly-α-olefin and the fluidity improver as the component (B) is improved. This effect is especially remarkable with the use of a polyoxyalkylene glycol compound as the fluidity improver.

On the other hand, the fluidity improver acts to improve the fluidity of a hydrocarbonic compound at low temperatures (those of the evaporator) in the presence of a small amount of substitute flon refrigerant such as R-134a, so as to provide good returnability of the lubricant in the refrigerating cycle. The kinematic viscosity of the fluidity improver is not particularly limited but is ordinarily 2 to 100cSt, preferably 3 to 50cSt at 40°C.

A typical example thereof is a polyoxyalkylene glycol compound. Various polyoxyalkylene glycol compounds can be used and an appropriate one may be selected from them according to the intended use. Preferred among them is a polyoxyalkylene glycol compound represented by the general formula (I): wherein R¹ is a hydrogen atom, an alkyl group having 1 to 10 carbon atoms, an alkenyl group having 2 to 10 carbon atoms, an alkynyl group having 2 to 10 carbon atoms, an aryl group having 6 to 10 carbon atoms, an aralkyl group having 7 to 10 carbon atoms, an acyl group having 2 to 10 carbon atoms or an aliphatic hydrocarbon group having 2 to 6 bonding links; R² is an alkylene group having 2 to 6 carbon atoms; R³ is a hydrogen atom, an alkyl group having 1 to 10 carbon atoms, an alkenyl group having 2 to 10 carbon atoms, an alkynyl group having 2 to 10 carbon atoms, an aryl group having 6 to 10 carbon atoms, an aralkyl group having 7 to 10 carbon atoms or an acyl group having 2 to 10 carbon atoms; n is an integer of 1 to 6; and m is a figure satisfying that the average value of mxn is 2 to 40.

The alkyl group having 1 to 10 carbon atoms may be straight chain, branched chain or cyclic. Specific examples of the alkyl group include a methyl group, an ethyl group, a n-propyl group, an isopropyl group, various butyl groups, various pentyl groups, various hexyl groups, various heptyl groups, various octyl groups, various nonyl groups, various decyl groups, a cyclopentyl group, a cyclohexyl group, a phenyl group, a tolyl group, a xylyl group, a benzyl group, a phenethyl group and the like.

An alkyl group having more than 10 carbon atoms leads to the degradation of the effect on improving the fluidity of the lubricant. The alkyl group has preferably 1 to 6 carbon atoms.

An alkyl moiety of said acyl group may be straight chain, branched chain or cyclic. Specific examples of the alkyl moiety of the acyl group include a methyl group, an ethyl group, a n-propyl group, an isopropyl group, various butyl groups, various pentyl groups, various hexyl groups, various heptyl groups, various octyl groups, various nonyl groups, a cyclopentyl group, a cyclohexyl group and the like. An acyl group having more than 10 carbon atoms leads to the degradation of the effect on improving the fluidity of the lubricant. The acyl group has preferably 2 to 6 carbon atoms.

Said R¹ and R³ may be same or different one another.

Furthermore, a plurality of R³s in a molecule may be same or different when n is 2 or more.

When R¹ is an aliphatic hydrocarbon group having 1 to 10 carbon atoms and 2 to 6 bonding links, the aliphatic hydrocarbon group may be either chain or cyclic. Examples of the aliphatic hydrocarbon group having 2 bonding links include an ethylene group, a propylene group, a butylene group, a pentylene group, a hexylene group, a heptylene group, an octylene group, a nonylene group, a decylene group, a cyclopentylene group, a cyclohexylene group, a vinyl group, an allyl group, a butenyl group, an ethynyl group, a propynyl group, and the like. Examples of the aliphatic hydrocarbon group having 3 to 6 bonding links include a residue after a hydroxyl group is removed from a polyhydric alcohol such as trimethylolpropane, glycerin, pentaerythritol, d ipentaerythritol, sorbitol, 1,2,3-trihydroxycyclohexane and 1,3,5-trihydroxycyclohexane.

An aliphatic hydrocarbon group having more than 10 carbon atoms leads to the degradation of the effect on improving the fluidity of the lubricant. The aliphatic hydrocarbon has preferably 2 to 6 carbon atoms.

R² of said general formula (I) is an alkylene group having 2 to 6 carbon atoms and examples of the oxyalkylene group as a repeating unit include an oxyethylene group, an oxypropylene group, an oxybutylene group, an oxypentylene group and an oxyhexylene group. A molecule thereof may comprise either same oxyalkylene groups or two or more different kinds of oxyalkylene groups. Preferably a molecule thereof comprises the alkylene groups each having at least 3 carbon atoms, more preferably 50% or more by mole of the alkylene groups each having at least 4 carbon atoms per oxyalkylene unit.

n of said general formula (I) is an integer of 1 to 6 and depends on the number of bonding links of R¹. For example, when R¹ is a hydrogen atom, an alkyl group, an alkenyl group, an alkynyl group, an aryl group or an acyl group, n is 1. When R¹ is an aliphatic hydrocarbon group having 2, 3, 4, 5 or 6 bonding links, n is 2, 3, 4, 5 or 6, respectively. Further, m is a figure satisfying that the average value of mxn is 2 to 40, and when the average value of mxn is out of said range, the object of the present invention is not achieved to a full extent.

Other than set forth above, examples of the polyoxyalkylene glycol compound for use in the present invention include a polyoxyalkylene glycol compound containing at least one constitutional unit represented by the general formula (II): wherein R⁴ is a monovalent hydrocarbon group having 1 to 10 carbon atoms and R⁵ to R⁹ are each a hydrogen atom or a monovalent hydrocarbon group having 1 to 10 carbon atoms.

Various polyoxyalkylene glycol compounds other than enumerated above can be used in the present invention as well, including those having a glycidyl group, those having a carbonyl bond in the molecule, those resulting from the substitution by a fluorine atom and the like.

Of above-mentioned polyoxyalkylene glycol compounds, a polyoxypropylene glycol compound, a polyoxybutylene glycol compound, a polyoxypentylene glycol compound and a polyoxyhexylene glycol compound are preferably used in the present invention because of their improvement in the mixing stability. Most suitable is a fluidity improver containing 50% or more of at least one compound selected from the group consisting of the polyoxybutylene glycol compound, the polyoxypentylene glycol compound and the polyoxyhexylene glycol compound. It is also preferable that a polyoxyalkylene glycol compound should contain the oxybutylene, oxypentylene and oxyhexylene units to foot up to 50 or more among oxyalkylene units forming the compound.

Furthermore, a polysiloxane compound such as dimethylpolysiloxane and a fluoride thereof can be used as the fluidity improver in the present invention as well. It is also effective to use a mixture of 2 or more different fluidity improvers.

The synthetic oil (A) and the fluidity improver (B) are mixed at a ratio by weight of 60 to 90% of (A) to 10 to 40%, respectively of (B).

When less than 5% by weight of the fluidity improver is used, the fluidity of the lubricant is undesirably not improved and therefore the sufficient returnability of the lubricant is not achieved as well. On the other hand, when more than 60% by weight of the fluidity improver is used, wear resistance and the like are undesirably degraded. This is accompanied by the degradation of the fundamental performance required for refrigerating machine lubricant, including the reduction of insulation resistance, worsening of hydrolytic stability, the increase in hygroscopicity and the like.

The lubricant of the present invention comprises as the essential component the base oil comprising the synthetic oil (A) and the fluidity improver (B) as set forth above and as the need arises various additives can be incorporated therein. Examples of the additive include an anti-wear additive such as phosphoric acid ester and phosphorous acid ester, an antioxidant, a chlorine scavenger, a metal deactivator, a defoaming agent, a detergent-dispersant, a viscosity index improver, a rust preventive, a corrosion inhibitor and the like.

As set forth above, the lubricant for refrigerating machines employing the refrigerant comprising tetrafluoroethane as claimed herein is excellent in the performance such as wear resistance, electrical insulating properties, hydrolytic stability, nonhygroscopicity and the like and further has excellent returnability of the lubricant. The lubricant of the present invention can be used along with a substitute flon refrigerant in a compression-type refrigerating cycle without a hitch.

The lubricant of the present invention is especially effective when used in automobile or household air conditioners, refrigerators and the like, having high industrial usefulness.

Next, the present invention will be described in greater detail below, with reference to non-limitative examples and comparative examples.

### Examples 1 to 6 and Comparative Examples 1 to 3

The synthetic oils and the fluidity improvers were each mixed as shown in Table 1 to prepare the lubricants for use in following tests. The results thereof are given in Table 2.

The lubricants were evaluated by determining each aspect of the performance thereof in accordance with the following test method:

### Evaluation of the performance

### (1) Fluidity of the lubricants at low temperatures

A lubricant mixed with 10% of R-134a was collected into a pressure glass tube having a diameter of 8mm, then a steel ball of 3/16in. (4.76 mm) in diameter was introduced therein and the pressure glass tube was sealed.

After the pressure glass tube was retained at -45°C, the steel ball was caused to fall to determine the time (second) required until the steel ball reached a point 10cm to 5cm above the bottom of the tube. The result thereof is given in terms of relative value.

### (2) Wear resistance

The wear test was conducted under the following conditions by using a Falex friction testing machine.

R-134a was blown at a rate of 5 liter/hour, and a test piece was subjected to wear for 60 minutes under a load of 300lbs (135.9 kg) and at 1,000rpm. Meanwhile, the test pieces such as block and pin were made of a standard material in accordance with ASTM D-3233.

Standard of evaluation (wear amount)
- ○:: less than 6.0mg
- △:: 6.0mg or more to 15mg or less
- ×:: more than 15mg

### (3) Electrical insulating properties

The electrical insulating properties was evaluated mutatis mutandis according to JIS C-2101 to determine the volume resistivity (room temperature).

### (4) Hydrolytic stability

100g of a lubricant, 10g of R-134a, 5ml of water and copper and iron catalysts were placed in a pressure container having a capacity of 300cc. Then, the pressure container was sealed and retained at 100°C for 5 days and thereafter the rate of a rise in the total acid number was determined.

Standard of evaluation
- ○:: less than 0.01mgKOH/g
- Δ:: 0.01mgKOH/g or more to 0.1mgKOH/g or less
- ×:: more than 0.1mgKOH/g

### (5) Hygroscopicity

10g of a test sample was placed in a 50cc glass container having a diameter of 30mm⌀. The glass container was introduced into a thermostat-humidistat and allowed to stand for 5 days at a temperature of 25°C and under a humidity of 85% and thereafter the water content of the test sample was determined.

Standard of evaluation
- ○:: less than 0.03%
- Δ:: 0.03% or more to 0.1% or less
- ×:: more than 0.1%

## Claims

1. A lubricant for refrigerating machines employing a refrigerant comprising 1,1,1,2-tetrafluoroethane or 1,1,2,2-tetrafluoroethane which comprises as an essential component a base oil comprising (A) 60 to 90% by weight of a synthetic oil formed of a poly-α-olefin or a mixture of a poly-α-olefin and an alkylbenzene and (B) 10 to 40% by weight of a fluidity improver formed of at least one compound selected from the group consisting of a polyoxyalkylene glycol compound, and a polysiloxane compound.

2. A lubricant for refrigerating machines employing a refrigerant comprising 1,1,1,2-tetrafluoroethane or 1,1,2,2-tetrafluoroethane as disclosed in claim 1 which comprises as an essential component a base oil comprising (A) 60 to 90% by weight of a synthetic oil formed of a poly-α-olefin or a mixture of a poly-α-olefin and an alkylbenzene and (B) 10 to 40% by weight of a fluidity improver formed of a polyoxyalkylene glycol compound.

3. The lubricant according to Claim 1 or 2, wherein said poly-α -olefin is a polymer of an α-olefin having 8 to 14 carbon atoms and a kinematic viscosity of 10 to 350cSt at 40°C.

4. The lubricant according to Claim 3, wherein said polymer of an α-olefin is a polymer of 1-dodecene, 1-decene or 1-octene, each having a kinematic viscosity of 10 to 350cSt at 40 °C.

5. The lubricant according to Claim 1 or 2, wherein said alkylbenzene is selected from a soft alkylbenzene and a hard alkylbenzene, each having a kinematic viscosity of 10 to 350cSt at 40°C.

6. The lubricant according to Claim 1 or 2, wherein said mixture of the poly-α-olefin and the alkylbenzene has a poly-α-olefin content of 5 to 90% by weight of the mixture.

7. The lubricant according to Claim 1 or 2, wherein said fluidity improver as the component (B) has a kinematic viscosity of 3 to 50cSt at 40°C.

8. The lubricant according to Claim 1 or 2, wherein said polyoxyalkylene glycol compound is represented by the general formula (I):
R¹ [(OR²)ₘ OR³]ₙ (I)
wherein R¹ is a hydrogen atom, an alkyl group having 1 to 10 carbon atoms,an alkenyl group having 2 to 10 carbon atoms, an alkynyl group having 2 to 10 carbon atoms, an aryl group having 6 to 10 carbon atoms, an aralkyl group having 7 to 10 carbon atoms, an acyl group having 2 to 10 carbon atoms or an aliphatic hydrocarbon group having 2 to 6 bonding links; R2 is an alkylene group having 2 to 6 carbon atoms; R³ is a hydrogen atom, an alkyl group having 1 to 10 carbon atoms, an alkenyl group having 2 to 10 carbon atoms, an alkynyl group having 2 to 10 carbon atoms, an aryl group having 6 to 10 carbon atoms, an aralkyl group having 7 to 10 carbon atoms or an acyl group having 2 to 10 carbon atoms; n is an integer of 1 to 6; and m is a figure satisfying that the average value of m x n is 2 to 40.

9. The lubricant according to Claim 8, wherein said polyoxyalkylene glycol compound contains 50% or more by mole of alkylene groups each having at least 4 carbon atoms per oxyalkylene unit for each molecule.

10. The lubricant according to Claim 1 or 2, wherein said polyoxyalkylene glycol compound contains at least one constitutional unit represented by the general formula (II): wherein R⁴ is a monovalent hydrocarbon group having 1 to 10 carbon atoms; and R⁵ to R⁹ are each a hydrogen atom or a monovalent hydrocarbon group having 1 to 10 carbon atoms.

11. The lubricant according to Claim 8, wherein said polyoxyalkylene glycol compound is a polyoxypropylene glycol compound, a polyoxybutylene glycol compound, a polyoxypentylene glycol compound or a polyoxyhexylene glycol compound.

12. The lubricant according to Claim 1 or 2, wherein said fluidity improver of component (B) comprises 50% or more of at least one compound selected from the group consisting of a polyoxybutylene glycol compound, a polyoxypentylene glycol compound and a polyoxyhexylene glycol compound.

13. The lubricant according to Claim 1 or 2, wherein said polyoxyalkylene glycol compound contains oxybutylene units, oxypentylene units and oxyhexylene units to foot up to 50 or more among oxyalkylene units forming the compound.

14. A method for effecting lubrication in refrigerating machines employing a refrigerant comprising 1,1,1,2-tetrafluoroethane or 1,1,2,2-tetrafluoroethane wherein the lubricant of claim 1 or 2 is used.

15. A refrigerating system which comprises a compressor, a refrigerant comprising 1,1,1,2-tetrafluoroethane or 1,1,2,2-tetrafluoroethane, and a lubricant, said lubricant comprising a base oil according to any one of Claims 1 to 13.

16. A use of a lubricant according to claim 1 or 2 for effecting lubrication in refrigerating machines employing a refrigerant comprising 1,1,1,2-tetrafluoroethane or 1,1,2,2-tetrafluoroethane.

## Patentansprüche

1. Schmiermittel für Kältemaschinen, die ein Kältemittel verwenden, das 1,1,1,2-Tetrafluorethan oder 1,1,2,2-Tetrafluorethan umfaßt, welches als wesentliche Komponente umfaßt: ein Grundöl, das
(A) 60 bis 90 Gew.-% eines synthetischen Öls, das aus einem Poly-α-olefin oder einer Mischung eines Poly-α-olefins und einem Alkylbenzol gebildet wird, und
(B) 10 bis 40 Gew.-% eines Fluiditätsverbesserers umfaßt, der durch mindestens eine Verbindung gebildet wird, die aus der Gruppe augewählt wird, die aus einer Polyoxyalkylenglykolverbindung und einer Polysiloxanverbindung besteht.

2. Schmiermittel für Kältemaschinen, die ein Kältemittel verwenden, das 1,1,1,2-Tetrafluorethan oder 1,1,2,2-Tetrafluorethan umfaßt, wie im Anspruch 1 beschrieben, das als wesentliche Komponente umfaßt: ein Grundöl, das
(A) 60 bis 90 Gew.-% eines synthetischen Öls, das aus einem Poly-α-olefin oder einer Mischung eines Poly-α-olefins und einem Alkylbenzol gebildet wird, und
(B) 10 bis 40 Gew.-% eines Fluiditätsverbesserers umfaßt, der aus einer Polyoxyalkylenglykolverbindung gebildet wird.

3. Schmiermittel nach Anspruch 1 oder 2, worin das genannte Poly-α-olefin ein Polymer eines α-Olefins mit 8 bis 14 Kohlenstoffatomen und einer kinematischen Viskosität von 10 bis 350 cSt bei 40°C ist.

4. Schmiermittel nach Anspruch 3, worin das genannte Polymer eines α-Olefins ein Polymer von 1-Dodecen, 1-Decen oder 1-Octen ist, die jeweils eine kinematische Viskosität von 10 bis 350 cSt bei 40°C besitzen.

5. Schmiermittel nach Anspruch 1 oder 2, worin das genannten Alkylbenzol ausgewählt wird aus einem weichen Alkylbenzol und einem harten Alkylbenzol, die jeweils eine kinematische Viskosität von 10 bis 350 cSt bei 40°C besitzen.

6. Schmiermittel nach Anspruch 1 oder 2, worin die genannte Mischung des Poly-α-olefins und das Alkylbenzols einen Poly-α-olefingehalt von 5 bis 90 Gew.-% der Mischung aufweist.

7. Schmiermittel nach Anspruch 1 oder 2, worin der genannte Fluiditätsverbesserer als Komponente (B) eine kinematische Viskosität von 3 bis 50 cSt bei 40°C besitzt.

8. Schmiermittel nach Anspruch 1 oder 2, worin die genannte Polyoxyalkylenglykolverbindung durch die allgemeine Formel (I) dargestellt wird:
R¹ [(OR²)ₘOR³]ₙ (I)
worin R¹ ein Wasserstoffatom, eine Alkylgruppe mit 1 bis 10 Kohlenstoffatomen, eine Alkenylgruppe mit 2 bis 10 Kohlenstoffatomen, eine Alkinylgruppe mit 2 bis 10 Kohlenstoffatomen, eine Arylgruppe mit 6 bis 10 Kohlenstoffatomen, eine Aralkylgruppe mit 7 bis 10 Kohlenstoffatomen, eine Acylgruppe mit 2 bis 10 Kohlenstoffatomen oder einer aliphatischen Kohlenwasserstoffgruppe mit 2 bis 6 Bindungsgliedern ist; R² eine Alkylengruppe mit 2 bis 6 Kohlenstoffatomen ist; R³ ein Wasserstoffatom, eine Alkylgruppe mit 1 bis 10 Kohlenstoffatomen, eine Alkenylgruppe mit 2 bis 10 Kohlenstoffatomen, eine Alkinylgruppe mit 2 bis 10 Kohlenstoffatomen, eine Arylgruppe mit 6 bis 10 Kohlenstoffatomen, eine Aralkylgruppe mit 7 bis 10 Kohlenstoffatomen oder eine Acylgruppe mit 2 bis 10 Kohlenstoffatomen ist; n eine ganze Zahl von 1 bis 6 ist; und m eine Zahl ist, die die Bedingung erfüllt, daß der Durchschnittswert von m x n von 2 bis 40 beträgt.

9. Schmiermittel nach Anspruch 8, worin die genannte Polyoxyalkylenglykolverbindung 50 % oder mehr pro Mol Alkylengruppen aufweist, die jeweils mindestens 4 Kohlenstoffatome pro Oxyalkyleneinheit je Molekül aufweisen.

10. Schmiermittel nach Anspruch 1 oder 2, worin die genannte Polyoxyalkylenglykolverbindung mindestens eine Aufbaueinheit enthält, die durch die allgemeine Formel (II) dargestellt wird: worin R⁴ eine monovalente Kohlenwasserstoffgruppe mit 1 bis 10 Kohlenstoffatomen ist; und R⁵ bis R⁹ jeweils ein Wasserstoffatom oder eine monovalente Kohlenwasserstoffgruppe mit 1 bis 10 Kohlenstoffatomen sind.

11. Schmiermittel nach Anspruch 8, worin die genannte Polyoxyalkylenglykolverbindung eine Polyoxypropylenglykolverbindung, eine Polyoxybutylenglykolverbindung, eine Polyoxypentylenglykolverbindung oder eine Polyoxyhexylenglykolverbindung ist.

12. Schmiermittel nach Anspruch 1 oder 2, worin der genannte Fluiditätsverbesserer der Komponente (B) 50 % oder mehr mindestens einer Verbindung umfaßt, die aus der Gruppe ausgewählt wird, die aus einer Polyoxybutylenglykolverbindung, einer Polyoxypentylenglykolverbindung und einer Polyoxyhexylenglykolverbindung besteht.

13. Schmiermittel nach Anspruch 1 oder 2, worin die genannte Polyoxyalkylenglykolverbindung Oxybutyleneinheiten, Oxypentyleneinheiten und Oxyhexyleneinheiten enthält, um bis zu 50 oder mehr unter den die Verbindungen bildenden Oxyalkyleneinheiten zu bilden.

14. Verfahren zur Schmierung in Kältemaschinen, die ein Kältemittel verwenden, das 1,1,1,2-Tetrafluorethan oder 1,1,2,2-Tetrafluorethan umfaßt, worin das Schmiermittel nach Anspruch 1 oder 2 verwendet wird.

15. Kältesystem, das einen Kompressor, ein Kältemittel, 1,1,1,2-Tetrafluorethan oder 1,1,2,2-Tetrafluorethan umfaßt, und ein Schmiermittel umfaßt, wobei das Schmiermittel das Grundöl nach irgendeinem der Ansprüche 1 bis 13 umfaßt.

16. Verwendung eines Schmiermittels nach Anspruch 1 oder 2 zur Schmierung von Kältemaschinen, die ein Kältemittel verwenden, das 1,1,1,2-Tetrafluorethan oder 1,1,2,2-Tetrafluorethan umfaßt.

## Revendications

1. Un lubrifiant pour des machines frigorifiques utilisant un réfrigérant comprenant du 1,1,1,2-tétrafluoroéthane ou du l,l,2,2-tétrafluoroéthane, qui comprend comme constituant essentiel une huile de base comprenant (A) 60 à 90 % en poids d'une huile synthétique formée d'une poly-alpha-oléfine ou d'un mélange d'une poly-alpha-oléfine et d'un alcoylbenzène et (B) 10 à 40 % en poids d'un agent améliorant la fluidité comprenant un composé choisi dans le groupe constitué par les polyoxyalcoylène glycols et les polysiloxanes.

2. Un lubrifiant pour des machines frigorifiques utilisant un réfrigérant contenant du 1,1,1,2-tétrafluoroéthane ou du 1,1,2,2-tétrafluoroéthane selon la revendication 1, qui comprend comme constituant essentiel une huile de base comprenant (A) 60 à 90 % en poids d'une huile synthétique formée d'une poly-alpha-oléfine ou d'un mélange d'une poly-alpha-oléfine et d'un alcoylbenzène et (B) 10 à 40 % en poids d'un agent améliorant la fluidité formé d'un polyoxyalcoylène glycol.

3. Un lubrifiant selon la revendication 1 ou 2, dans lequel la poly-alpha-oléfine est un polymère d'une alpha-oléfine ayant 8 à 14 atomes de carbone et une viscosité cinématique de 10 à 350 cSt à 40°C.

4. Un lubrifiant selon la revendication 3, dans lequel le polymère d'une alpha-oléfine est un polymère de 1-dodécène, de 1-décène ou de 1-octène, ayant chacun une viscosité cinématique de 10 à 350 cSt à 40°C.

5. Un lubrifiant selon la revendication 1 ou 2, dans lequel l'alcoylbenzène est choisi parmi un alcoylbenzène mou et un alcoylbenzène dur, ayant chacun une viscosité cinématique de 10 à 350 cSt à 40°C.

6. Un lubrifiant selon la revendication 1 ou 2, dans lequel le mélange de la poly-alpha-oléfine et de l'alcoyl benzène a une teneur en poly-alpha-oléfine de 5 à 90 % en poids par rapport au mélange.

7. Un lubrifiant selon la revendication 1 ou 2, dans lequel l'agent améliorant la fuidité utilisé comme constituant (B) a une viscosité cinématique de 3 à 50 cSt à 40°C.

8. Un lubrifiant selon la revendication 1 ou 2, dans lequel le polyoxyalcoylène glycol est représenté par la formule générale (I) :
R¹ ((OR²)ₘ OR³)ₙ (I)
où R¹ est un atome d'hydrogène, un groupe alcoyle ayant 1 à 10 atomes de carbone, un groupe alcényle ayant 2 à 10 atomes de carbone, un groupe alcynyle ayant 2 à 10 atomes de carbone, un groupe aryle ayant 6 à 10 atomes de carbone, un groupe aralcoyle ayant 7 à 10 atomes de carbone, un groupe acyle ayant 2 à 10 atomes de carbone ou un groupe d'hydrocarbure aliphatique ayant 2 à 6 liaisons d'enchaînement ; R² est un groupe alcoylène ayant 2 à 6 atomes de carbone ; R³ est un atome d'hydrogène, un groupe alcoyle ayant 1 à 10 atomes de carbone, un groupe alcényle ayant 2 à 10 atomes de carbone, un groupe alcynyle ayant 2 à 10 atomes de carbone, un groupe aryle ayant 6 à 10 atomes de carbone, un groupe aralcoyle ayant 7 à 10 atomes de carbone ou un groupe acyle ayant 2 à 10 atomes de carbone ; n est un nombre entier de 1 à 6 ; et m est un nombre tel que la valeur moyenne de m x n soit de 2 à 40.

9. Un lubrifiant selon la revendication 8, dans lequel le polyoxyalcoylène glycol contient 50 % ou plus, en moles, de groupes alcoylène ayant chacun au moins 4 atomes de carbone par maille oxyalcoylène pour chaque molécule.

10. Un lubrifiant selon la revendication 1 ou 2, dans lequel le polyoxyalcoylène glycol contient au moins une unité constitutive représentée par la formule générale (II) où R⁴ est un groupe d'hydrocarbure monovalent ayant 1 à 10 atomes de carbone et R⁵ à R⁹ sont chacun un atome d'hydrogène ou un groupe d'hydrocarbure monovalent ayant 1 à 10 atomes de carbone.

11. Un lubrifiant selon la revendication 8, dans lequel le polyoxyalcoylène glycol est un polyoxypropylène glycol, un polyoxybutylène glycol, un polyoxypentylène glycol ou un polyoxyhexylène glycol.

12. Un lubrifiant selon la revendication 1 ou 2, dans lequel l'agent améliorant la fluidité du constituant (B) comprend 50 % ou plus d'au moins un composé choisi dans le groupe constitué par les polyoxybutylène glycols, les polyoxypentylène glycols et les polyoxyhexylène glycols.

13. Un lubrifiant selon la revendication 1 ou 2, dans lequel le polyoxyalcoylène glycol contient des mailles oxybutylène, des mailles oxypentylène et des mailles oxyhexylène dans une mesure allant jusqu'à 50 ou plus parmi les mailles oxyalcoylène formant le composé.

14. Une méthode pour effectuer la lubrification dans des machines frigorifiques utilisant un réfrigérant contenant du 1,1,1,2-tétrafluoroéthane ou du 1,1,2,2-tétrafluoroéthane, dans laquelle on utilise le lubrifiant de la revendication 1 ou 2.

15. Un système frigorifique qui comprend un compresseur, un réfrigérant comprenant du 1,1,1,2-tétra fluoroéthane ou du l,l,2,2-tétrafluoroéthane et un lubrifiant, ce lubrifiant comprenant une huile de base selon l'une quelconque des revendications 1 à 13.

16. L'utilisation d'un lubrifiant selon la revendication 1 ou 2 pour effectuer la lubrification dans des machines frigorifiques utilisant un réfrigérant comprenant du l,l,l,2-tétrafluoroéthane ou du 1,1,2,2-tétrafluoroéthane.
